

## UNITED STATES PATENT OFFICE

2,024,014

## PROCESS FOR IMPROVEMENT OF MALLEABLE IRON CASTINGS

Cyril Stanley Smith, Cheshire, Conn., assignor, by mesne assignments, to Battelle Memorial Institute, Columbus, Ohio, a corporation of Ohio

No Drawing. Application October 13, 1932,  
Serial No. 637,671

8 Claims. (Cl. 148—21.8)

This invention relates to the production of malleable iron castings of superior strength, the improvement resulting from the addition of a substantial amount of copper combined with a process of heat treatment, following the usual malleabilizing anneal, which has for its object the dispersion of the copper in a suitable sub-microscopic form to cause the so-called precipitation hardening.

10 In the production of malleable iron castings the customary method consists of making white-fracture iron castings from a molten metal containing 2 to 3 percent carbon, 0.8 to 2 percent silicon, with small amounts of manganese and traces 15 of sulphur and phosphorus. The composition is adjusted so that the castings contain substantially all the carbon in the combined form and are very hard and brittle. The castings are then annealed for prolonged periods at temperatures 20 customarily in the neighborhood of 850 to 950° C. to cause the undissolved combined carbon or iron carbide to change to graphite and cooled slowly to a temperature below the critical point. Various modifications of this process resulting in a 25 shorter time have been proposed, but all have for their object the production of a final microstructure consisting of rounded particles of temper carbon embedded in a soft iron matrix with practically no combined carbon. Metal having this 30 structure possesses considerable ductility.

In its broadest aspects the invention comprises the precipitation hardening of malleable cast iron by the addition of any element whose solubility in alpha iron or iron below the critical point increases with an increase in temperature. The 35 hardening results from a heat treatment comprising heating to a temperature where a substantially greater amount of the added element is dissolved than is soluble at room temperature, cooling 40 at a rate sufficient to retain the excess of the added element in solution, and reheating to a temperature at which precipitation of the element will occur. Under suitable conditions of dispersion the precipitation will result in considerable hardening. I have found copper to be a 45 very suitable element to use in securing the precipitation hardening.

I have found that copper up to about 5 percent may be incorporated with the molten metal before casting without harmful effect on the process of malleabilizing or graphitizing, but the finally malleabilized casting can then be greatly improved by giving a so-called precipitation hardening treatment, that is, a heat treatment to dissolve the copper and, according to the present

accepted theory, reprecipitate it in a sub-microscopic form of such a nature that the soft iron matrix is considerably strengthened without very much loss of ductility. In its essentials, the heat treatment consists of heating the copper-containing malleable casting to a suitable temperature for sufficient time to dissolve a large amount of the copper (a heat treatment hereinafter referred to as the solution heat treatment) cooling at a rate sufficiently great to retain most of the copper in solution and then reheating to an intermediate temperature for sufficient time to enable the excess copper to be thrown out of solution in a critically dispersed condition, to produce substantially maximum hardening.

The molten iron used for the production of castings under this invention may be of any composition which will give an annealable white iron casting, employing either sand or permanent molds, and is distinguished from that used in customary practice by the addition of copper in amounts sufficient to respond to the precipitation hardening treatment.

The smallest amount of copper which will result in precipitation hardening is about 0.6 percent and, while the maximum effect occurs at 1 to 1.5 percent copper, for some purposes it may be desirable to have as much as 5 percent copper, although for most purposes it probably would not be desirable to go above about 3 percent. The 25 white iron castings containing copper may be rendered malleable by any of the customary graphitizing processes; either the slow treatment in which the castings, usually packed in boxes and supported in scale, sand or other oxidizing 30 or non-oxidizing packing material, are subjected to a cycle of heating to a temperature above the critical temperature ( $A_1$ ) and very slow cooling to a temperature below the critical temperature, or any of the recently developed short cycle processes which by a suitable control of the temperature complete graphitization much more rapidly. In any case, save for the somewhat shorter time required when copper is present, the treatment 40 up to this point is indistinguishable from the 45 customary methods and the product is a malleable casting distinguished only by a slightly greater strength and better corrosion resistance on account of its copper content. Microscopically the 50 structure of the malleable iron in this stage consists of ferrite, temper carbon (graphite), and copper which is distributed in the form of microscopically visible particles scattered throughout the ferrite in amounts depending upon the excess of the copper content above the solid solu- 55

5 ability of copper in ferrite at the lowest temperature of the malleabilizing process. There may also be small quantities of pearlite or cementite if the malleabilization was accidentally or intentionally stopped before graphitization was complete. The presence of the copper particles is all that distinguishes the microstructure of the metal from ordinary malleable iron in this stage.

10 In my invention the complete malleabilized iron containing copper is then given a final heat treatment to develop precipitation hardening. The malleabilized castings are heated to a temperature at which a substantial portion of the copper will be redissolved in solid solution, which temperature may preferably be in the range from 15  $700^{\circ}$  to  $850^{\circ}$  C. ( $1290$  to  $1565^{\circ}$  F.) and then quenched, air cooled or cooled by other means but at a rate faster than approximately  $25^{\circ}$  C. 20 ( $45^{\circ}$  F.) per hour to a temperature below approximately  $600^{\circ}$  C. and which may be to approximately room temperature, and reheated or maintained for a suitable length of time at a temperature in the range of  $400$  to  $600^{\circ}$  C. ( $750$  to 25  $1110^{\circ}$  F.) followed by final cooling at any speed to room temperature. The first stage of this process, by putting copper in solution, strengthens the iron appreciably but the greatest increase in 30 strength occurs during the precipitation treatment and the final product has a substantially higher strength than metal not containing copper but otherwise of identical composition subjected to the same heat treatment, or than metal containing copper which has not been subjected to 35 the heat treatment described.

As a specific example of the improvement due to the process, the following results of mechanical tests are given. The two cast irons were of practically identical composition save for the presence 40 of one percent copper in melt B.

## **Change in properties of malleable iron due to heat treatment**

| 45  | Temperature of solution heat treatment <sup>1</sup> | Melt "A"<br>0.0 percent copper |                              | Melt "B"<br>1.0 percent copper |                              |
|-----|-----------------------------------------------------|--------------------------------|------------------------------|--------------------------------|------------------------------|
|     |                                                     | Increase in yield point        | Increase in tensile strength | Increase in yield point        | Increase in tensile strength |
| 50  | ° C.                                                | lbs./sq. in.                   | lbs./sq. in.                 | lbs./sq. in.                   | lbs./sq. in.                 |
| 700 | 700 R.H.                                            | 2,450                          | 1,500                        | 1,700                          | 4,750                        |
| 730 | 730 R.H.                                            | 2,550                          | 2,100                        | 3,050                          | 3,300                        |
| 740 | 740 R.H.                                            | 2,850                          | 400                          | 5,650                          | 5,100                        |
| 55  | 750 R.H.                                            | 450                            | 500                          | 3,150                          | 3,800                        |
| 775 | 775 R.H.                                            | 550                            | 400                          | 14,850                         | 8,500                        |
| 800 | 800 R.H.                                            | 1,550                          | 1,700                        | 1,750                          | 1,700                        |
| 800 | 800 R.H.                                            | 1,550                          | 1,000                        | 11,350                         | 6,000                        |
| 60  | 860 R.H.                                            | 1,550                          | 2,800                        | 3,350                          | 8,900                        |
|     |                                                     | 750                            | 1,300                        | 15,950                         | 20,700                       |
|     |                                                     | 11,550                         | 21,900                       | 12,650                         | 26,300                       |
|     |                                                     | 12,050                         | 24,100                       | 28,350                         | 40,100                       |
|     |                                                     | 25,950                         | 37,400                       | 32,850                         | 44,900                       |
|     |                                                     | 28,550                         | 46,300                       | 42,350                         | 56,500                       |

<sup>1</sup> Solution heat treatment was followed by air cooling. RH indicates sample reheated 4 hours at 500°C.

65 The temperature of the solution heat treatment must be high enough to dissolve a substantial amount of copper, at least above  $730^{\circ}$  C. in the iron considered above, but this will vary with composition. Greater ductility will result if the temperature is below the critical point (about  $760^{\circ}$  C. in most malleable iron, somewhat less when copper is present) and if this is exceeded the resulting re-solution of carbon will result in a further increase of strength but with loss of ductility. It is an advantage to use a reasonably high temperature to obtain sufficient copper in solution.

70

75

and a small amount of carbon re-solution resulting in the final production of pearlitic or sorbitic patches scattered throughout the structure is not harmful and for some uses may be definitely advantageous.

Microscopically, the precipitation hardening described does not change the structure other than by causing the disappearance of the fine copper particles existing in the malleabilized material. The cooling is sufficiently rapid to prevent visible precipitation of copper and the final precipitation heat treatment at about 500° C. causes a change which is quite invisible under the microscope. Treatment above the critical point dissolves some carbon which diffuses and gives rise to pearlitic patches on cooling, but the main purpose of the invention is to cause precipitation of the copper, regardless of pearlite formation. 10 13

It will be obvious to one skilled in the art that 20 a number of modifications of the heat treating process described are possible, and it should be understood that this invention is not restricted to the simple air cooling and reheating treatment described above, but any modification of 25 this procedure that has for its aim the precipitation hardening of the metal by suitable dispersion of the copper is covered by the present invention. For instance, it is unnecessary to cool the malleabilized castings to room temperature before heat treatment, but the castings—either in a separate furnace or in the one used for the malleabilizing anneal—may be heated directly from the final malleabilizing temperature to the proper temperature for putting the copper into 30 solution, and the process thereafter continued as described by cooling and reheating. A sample malleabilized and then directly heated from the final malleabilizing temperature to 745° C., maintained for one hour and air cooled had a Brinell 35 hardness number of 120. On reheating the sample for four hours at 500° C. to cause precipitation the hardness increased to 138, showing that the solution heat treatment may follow the malleabilizing treatment directly without intermediate cooling and without appreciable effect on the properties. I have also found that it is unnecessary to cool to room temperature from the solution heat treatment, whether this follows directly the malleabilizing or follows cooling to room 40 temperature, but the cooling may be stopped at the desired temperature and the precipitation treatment continued directly thus saving both heat and time. As a specific example, a sample of cast iron containing one percent copper was 45 malleabilized by a suitable treatment and the temperature raised directly without intermediate cooling to 745° C., held one hour to permit 50

the copper to dissolve, withdrawn from the furnace and cooled in the air to about 500° C., when it was placed in a second furnace maintained at about 500° C., held at this temperature for four hours and finally cooled to room temperature. This sample, which had not been cold from the time of charging in the malleabilizing furnace to the end of the precipitation treatment, had a Brinnell hardness of 142, equal to that obtained by an intermittent process.

The proper duration of the precipitation treatment depends on the temperature and if the proper combination of time and temperature is exceeded the metal softens again. At 450° C. about 24 hours, at 500° C. about 4 hours, and at 550° C. about 2 hours suffice, while at 600° C. about 15 minutes give maximum hardness, and 75

further time results in softening. There is an advantage in using a low temperature of precipitation not only on account of the easier controllability of the time but also because the resulting properties are somewhat better, but commercial operations may well require the shorter time of treatment resulting from the use of higher temperatures.

It will sometimes prove advisable to quench the specimens rather than to air cool them following the solution heat treatment, but in general I prefer to air cool since this is sufficiently rapid to retain most of the copper in solution and it avoids the danger of warping which exists when castings of complicated sections are quenched. The castings may also be cooled from the solution heat treatment in a furnace or by any other means provided that the rate of cooling above about 500° C. is not less than approximately 25° C. per hour. When it is desired to give the precipitation treatment directly without cooling to room temperatures, a molten bath of fusible salt or metal maintained at the desired precipitation temperature may be used to obtain rapid cooling.

Having thus set forth the nature of my invention, what I claim is:

1. The process for the heat treatment of malleable iron castings containing 0.6 to 5 percent copper comprising heating the malleabilized castings to a temperature in the range of approximately 700 to 850° C.; cooling at a rate greater than approximately 25° C. per hour to a temperature in the range of approximately 400 to 600° C.; and without further cooling maintaining in that temperature range for sufficient time to produce a substantial increase in hardness.

2. The process for the production of malleable iron castings comprising making castings from a white iron containing 0.6 to 5 percent copper; annealing the castings to convert substantially all the carbon into the uncombined state; raising the temperature into the range of approximately 700 to 850° C.; cooling at a rate greater than approximately 25° C. per hour to a temperature in the range of approximately 400 to 600° C.; and without further cooling maintaining in that temperature range for sufficient time to produce a substantial increase in hardness.

3. The process for the heat treatment of white iron castings containing 1.75 to 3.0 percent carbon, 0.6 to 2.5 percent silicon, 0.6 to 5 percent copper, the balance principally iron, comprising heating the castings to a temperature above the carbon critical point,  $A_1$ , for a sufficient time to convert substantially all the undissolved combined carbon to the form of temper carbon; cooling to a temperature below  $A_1$  and holding for a time sufficient to convert substantially all of the remaining carbon to the form of temper carbon; without further cooling heating to a temperature in the range of 700 to 850° C.;

cooling to a temperature of 400 to 600° C. and without further cooling maintaining in this temperature range for a time sufficient to produce an increase in hardness and tensile strength.

4. The process for the heat treatment of white iron castings containing 2.0 to 2.5 percent carbon, 0.8 to 1.2 percent silicon and about 1 percent copper, comprising annealing the castings to convert substantially all of the carbon to the form of temper carbon; reheating to a temperature of from about 745° C. to about 800° C.; cooling faster than about 25° C. per hour to a temperature in the neighborhood of 500° C. and without further cooling maintaining at this temperature until an appreciable increase in hardness has occurred.

5. The process for the production of malleable iron castings comprising incorporating from about 0.6 to about 5 percent copper with the molten iron before pouring, malleabilizing the castings, heating to a temperature range of 700 to 850° C., cooling at a rate faster than about 25° C. per hour to a temperature of 400 to 600° C., and without further cooling maintaining at a temperature of 400 to 600° C. for sufficient time to produce an increase in hardness and tensile strength.

6. The process for the production of malleable iron castings comprising making castings from white iron containing from about 0.6 to about 5 percent copper, annealing the castings to convert substantially all of the carbon into the uncombined state, heating to a temperature in the range of 700 to 850° C., cooling faster than a rate of about 25° C. per hour to a temperature of 400° to 600° C., and without further cooling maintaining at a temperature of 400 to 600° C. for a sufficient time to produce an increase in hardness and strength.

7. The process for the production of malleable iron castings comprising making white iron castings containing approximately 1 percent copper, annealing the castings to convert substantially all of the carbon to the form of temper carbon, heating to a temperature of about 745° C., cooling faster than about 25° C. per hour to a temperature in the neighborhood of 500° C., and without further cooling maintaining at a temperature in the neighborhood of 500° C. for about four hours.

8. The process for the heat treatment of malleable iron castings containing approximately 1% to 1.5% copper, comprising heating the malleabilized castings to a temperature in the range of 700 to 850° C., cooling at a rate greater than approximately 25° C. per hour to an approximate range of 400 to 600° C., and without further cooling maintaining in that temperature range for a sufficient length of time to produce a substantial improvement in properties.

CYRIL STANLEY SMITH.